

June 18, 1929.

W. H. FLOOD

1,717,445

PAVEMENT

Filed March 22, 1926



2



4



INVENTOR

Walter H. Flood

*Charles H. Flood*

Ex

Atty's

## UNITED STATES PATENT OFFICE.

WALTER H. FLOOD, OF CHICAGO, ILLINOIS.

## PAVEMENT.

Application filed March 22, 1926. Serial No. 96,366.

This invention relates to pavements and more particularly to a combination asphalt and concrete pavement and a method of forming the same.

5 The ordinary asphalt pavement has several defects, the most serious of which is its tendency to displacement resulting in waves and ruts. In order to overcome this fault, it is necessary that the percentage of asphalt be maintained within close limits and that the grading of the mineral aggregate be carefully controlled. In the less expensive form of asphalt paving, known as asphaltic concrete containing from 20 to 70% of 10 stone, the remainder being sand and asphalt, the displacement of the pavement is frequently due to the mortar of sand and asphalt preventing the stone particles from obtaining a firm bearing on each other. Greater 15 stability is secured when the stone particles are keyed together on themselves, the mortar functioning only to fill interstices or voids. It is, however, impossible to secure this condition by ordinary methods where all the ingredients are mixed together.

20 The advantages of an asphalt pavement are its plasticity, pliability, non-rigidity, resilience and ease of repair. The defects of cement concrete type of pavement are its rigidity and tendency to crack and disintegrate from stresses imparted by the sub-grade and temperature changes.

It is therefore an object of this invention 25 to provide a pavement that shall combine the advantages of asphalt and concrete pavements, but overcome their faults.

It is a further object of this invention to provide a pavement comprising crushed rock previously coated with asphalt and then 30 rolled or tamped into a coherent yet porous layer, the spaces between said rock being subsequently filled by a cement grout, whereby the rock is rigidly held in place yet sufficient 35 resiliency is provided by the asphalt to allow 40 for expansion and compression stresses.

It is a further important object of this invention to provide a method for forming a pavement of combination asphalt and concrete that shall possess the desired properties, resiliency and great stability.

Other and further important objects of this invention will be apparent from the disclosures in the specification and the accompanying drawings.

55 This invention (in a preferred form) is

illustrated in the drawings and hereinafter more fully described.

## On the drawings:

Figure 1 is a sectional view of a pavement, embodying the principles of my invention, 60 in the process of construction.

Figure 2 is an enlarged detail sectional view of the same.

Figure 3 is a sectional view of a pavement 65 in completed form.

Figure 4 is an enlarged detail sectional view of the same.

## As shown on the drawings:

My invention in general consists in first laying to the desired depth a layer of crushed 70 stone, indicated by the reference numeral 1, to which has preferably been previously applied a coating 2 of asphalt or similar bituminous compound over the individual particles of stone. The crushed stone 1 should be relatively coarse and preferably be previously graded from about 1½ inches in size down to ¼ or ⅛ inch, but with sufficient of the larger sizes to leave the finished mixture after rolling on the road bed 6 in an open condition. 75 The mixture may, if desired, contain some sand or fine material, but not enough to prevent the pieces of stone from bearing on each other firmly. The coating of asphalt 2 is only sufficient to thoroughly cover the individual 80 stones without filling up the voids 4 between the stones.

After spreading the asphalt stone mixture on the road bed and rolling it in in the customary way, a grout 3 of hydraulic cement 90 and water, with or without sand, is spread over the asphalt course and forced into it by means of squeegees, rollers or other suitable means so that all or nearly all of the interstices 4 in the asphalt mixture are filled. The 95 excess is then removed to form a smooth surface 5 and the cement mixture allowed to harden in the usual way. After hardening, the pavement may be opened to traffic, or if desired, a thin coating of asphalt cement may 100 be spread, followed by a coat of sand or stone chips which are then rolled in.

The grout of hydraulic cement may be made of any desired consistency, depending upon the conditions to be met. It will be 105 noted that the function of this grout is to produce a sort of artificial stone in the voids 4 between the particles of asphalt coated stone 1 and is not used as a cementing agent to hold the stone together as in the ordinary 110

concrete pavement. The asphalt coating 2 on the stone prevents any adhesion of the 3 grout to the stone. The grout forms a sort 5 of frame work or skeleton to firmly hold the 10 stone in position and prevent displacement but allows a slight movement of the stone 15 from expansion and contraction stresses due to temperature and other causes. It, therefore, does not result in a rigid pavement but 20 is made up of individual particles cemented together by the asphalt and made dense and 25 resistant to the entrance of water by means of the cement grout which forms artificial stone 30 particles, the exact size of the voids in the 35 asphalt mixture. In this manner a pavement 40 of great stability is secured which also 45 possesses resiliency and plasticity and is non-rigid.

It is not new to make a cement concrete 50 pavement by rolling the stone on the street and pouring a cement grout into and over the 55 stone. This, however, cements all particles together into a rigid slab producing a pavement 60 very similar to the ordinary concrete pavement. The advantage claimed for this 65 method over the ordinary manner of mixing all the materials together in a concrete mixer is that it is claimed to produce a denser and 70 stronger slab. The function of the cement 75 grout in this type of construction is, as pointed out, entirely different from that as employed in my invention.

As mentioned previously, an asphalt pavement must be closely controlled as to its 80 asphalt content; a slight excess results in an 85 unstable mixture with consequent displacement under traffic while a slight deficiency causes a tendency to cracking and disintegration 90 due to there not being sufficient asphalt 95 to cement the mineral aggregate firmly together. If it were not for the tendency to 100 displacement, which is the most common and serious fault of an asphalt pavement, a large amount of asphalt cement in the mixture 105 would be beneficial as it increases the pliability and resiliency of the pavement and its 110 resistance to the action of water.

This invention permits a wide range of 115 asphalt content and allows the use of a rich 120 mixture (that is, high in asphalt) as the cement grout supports the stone in its proper 125 place, thus preventing movement under traffic. In the asphalt mixture employed in this invention any kind of mineral aggregate 130 of suitable hardness may be used, such as gravel, slag, limestone, traprock, granite, and the like, and the mixture may be produced in the ordinary asphalt plant by heating the ingredients or any of the so-called cold processes may be used. In the cement grout any hydraulic cement may be used and if quick hardening is desired, the high alumina cements may be employed.

The essential elements of the invention are 135 an asphalt coated stone mixture in which the

stone is large enough to possess great stability and the subsequent filling of the voids in the asphalt mixture with artificial stone made by the hydraulic cement grout. As pointed out, it is necessary that the stone particles of asphalt mixture are thoroughly keyed together 70 and have a firm bearing on each other. This is a recognized practice in road construction, as in the building of water bound macadam pavements coarse stone is thoroughly rolled 75 until a good keying is secured, after which the voids are filled with fine stone screenings, water being used to secure thorough distribution of the screenings. In the ordinary type 80 of asphaltic concrete pavement, sand or fine aggregate must be mixed with the asphalt and stone in order to make the pavement close sufficiently to prevent water and dirt from entering and also to prevent movement of 85 the stone particles. As this sand is mixed with the stone and asphalt at the asphalt plant, it is impossible to retain the sand or finer particles entirely in the voids but much 90 of it gets between the stone particles and prevents a firm bearing and keying together 95 of the stone. In this invention the grout finds its way into the open voids and cannot prevent the stones from bearing on each other as they are already in proper position. It is a well known fact that the larger stone particles possess greater stability in the pavement than the small size. However, in an asphaltic concrete, the size of the stone is 100 limited on account of the large voids which the larger stone has so that the larger the particles of stone used the less amount of stone can be used as it requires more fine material to fill the voids. With this invention, stone of any size may be used, voids being 105 entirely filled by the cement grout.

It will of course be understood that tar or other bituminous compounds might be used in lieu of asphalt and by the use of the term asphalt herein I also intend to include tar and similar bituminous compounds.

I am aware that many changes may be made, and numerous details of construction may be varied through a wide range without departing from the principles of this invention, and I therefore do not purpose limiting the patent granted hereon, otherwise than necessitated by the prior art.

I claim as my invention:

1. A pavement comprising a course of stones individually coated with bituminous material of sufficient thickness to prevent adhesion of cement to the stones, and a hydraulic cement grouting for filling substantially all the voids in and the interstices between the stones of said course thus forming a skeleton framework for holding the stones in position and to prevent their displacement, said coating of bituminous material serving to bind the stones to the grouting as well as a partition medium to separate the stones 130

from the cement so as to allow for expansion and compression stresses and to thus minimize cracking of the pavement.

2. The process of laying a pavement which 5 consists in grading a given batch of stones, covering each of said stones with a bituminous material of sufficient thickness to prevent adherence of cement to the stones and to allow for expansion and compression 10 stresses to which the pavement may be subjected, laying a course of said stones, compacting said course so that the stones are keyed to each other to form a firm founda-

tion, spreading over said course and forcing thereinto a hydraulic cement grouting to substantially fill all the interstices and voids between the compact stones thus forming a skeleton framework for holding the stones in position and to prevent their displacement, and thereafter smoothing off an excess of 20 said cement grouting from the top of said stones.

In testimony whereof I have hereunto subscribed my name.

WALTER H. FLOOD.